

A. ROJEKOFF.

MOLD FOR PRODUCING COMPOSITE METAL CASTINGS.

APPLICATION FILED JULY 24, 1914.

1,151,398.

Patented Aug. 24, 1915.



WITNESSES

Geophmataz.  
M. S. Jers

INVENTOR  
Alexander Rojeckoff  
BY  
A. J. Dunn  
ATTORNEY

# UNITED STATES PATENT OFFICE.

ALEXANDER ROJEKOFF, OF BIEJITZA, RUSSIA.

## MOLD FOR PRODUCING COMPOSITE METAL CASTINGS.

1,151,398.

Specification of Letters Patent. Patented Aug. 24, 1915.

Original application filed September 18, 1912, Serial No. 720,953. Divided and this application filed July 24, 1914. Serial No. 852,818.

To all whom it may concern:

Be it known that I, ALEXANDER ROJEKOFF, a subject of the Emperor of Russia, residing at Biejitz, Russia, have invented certain new and useful Improvements in Molds for Producing Composite Metal Castings, of which the following is a specification.

My invention relates to steel castings composed of a plurality of various layers of steel, that is, layers having a different chemical composition, such as described in my application Serial No. 720,953, filed on September 18th, 1912, of which application, this application is a division.

The particular object of this invention is to provide means for producing perfect castings of this kind, made up of a number of concentric layers. By perfect castings, I mean castings which are free from blow holes, cracks or other defects. For making a casting of this kind a mold is used with partitions placed in the mold of polygonal or circular cross section. In order to produce a successful casting, these partitions must be split so that upon coming in contact with the hot fluid metal, they can expand without subjecting the casting, as it is allowed to cool, to undue strains, whereby cracks would be formed in the casting and the casting would be spoiled.

In the accompanying drawing, I have shown a mold in plan view with two partitions placed therein to illustrate my invention.

In the construction of the mold shown in the drawing by way of example, the mold proper is designated by the numeral 1, and is provided with the trunnions 2 and 3 arranged at opposite sides of the mold. In the mold are placed two partitions 4, 5, the former partition being of polygonal and the partition 5 being of circular cross section. The partition 4 is split at 4' and the partition 5 at 5', in such a way that the free edges of each partition overlap, a small space being left between these edges. Thus, three compartments are formed by these partitions, A. B. and C., and by means of such a mold a composite casting can be produced, made up of three layers, each layer having a different chemical composition.

The partitions are made of such a thickness, as to prevent the molten liquid mass

of steel, poured into one of the compartments, from mingling with the molten liquid 55 mass poured into the adjacent compartment. The thickness of the partitions must be determined by the temperature of the molten steel, as well as by the cross section of the casting to be produced. If the partitions 60 did not have the required thickness, the liquid molten steel of one compartment would melt the partition and mingle with the molten mass in the adjacent compartment, whereas, if the thickness of the partitions were too great, the partitions would not, as they should, properly combine with the molten liquid steel, in which case, of course, the casting would not be a uniformly fused mass. I find that in order to make a 70 perfect casting of this kind, the partitions should have a thickness of no less than 1% and no more than 3.8% of the cross section of the entire casting.

Due to the fact that the partitions are 75 split and a space is left between the overlapping free edges, the partitions on coming in contact with the hot liquid steel can freely expand, without subjecting the layers, during the cooling period, to undue strains. 80

It is a matter of great importance that the partitions should completely combine with the molten liquid steel of each compartment and in order to prevent the free edges of the partitions from projecting beyond the 85 individual castings, the thickness of the partitions along these edges is preferably reduced, as clearly shown in the drawing. With the partitions thus arranged and shaped, they can, not only freely expand, 90 due to the heat of the molten liquid metal, but they also can uniformly combine with the molten metal and thus a perfect casting, made up of various layers of steel having different chemical compositions, is produced. 95

The molten masses of steel preferably enter the various compartments from the bottom of the mold as is well known in the making of castings.

While I have shown in the drawing a 100 mold with two partitions of different cross sections, I wish it to be distinctly understood that my invention is not limited, of course, to any particular number of partitions, nor to a particular cross section and 105 I use the term "polygonal" in a broad sense

to also include partitions of circular cross section.

I claim:

In a mold for producing composite metal castings made up of layers having different chemical compositions, the combination with the mold of a number of split metal partitions of polygonal cross section, their edges

overlapping each other, and being free to move relative to each other. 10

In testimony whereof I have affixed my signature in presence of two witnesses.

ALEXANDER ROJEKOFF.

Witnesses:

ALEXANDER TSCHENALOFF,  
H. A. LOVIAGUINE.

Copies of this patent may be obtained for five cents each, by addressing the "Commissioner of Patents, Washington, D. C."